

## UNITED STATES PATENT OFFICE

WILLIAM H. HILL, OF ARLINGTON, NEW JERSEY, ASSIGNOR TO THE KOPPERS COMPANY OF DELAWARE, A CORPORATION OF DELAWARE

## COMPOSITION OF MATTER AND PROCESS OF PREPARING THE SAME

No Drawing. Application filed September 16, 1929. Serial No. 393,115.

This invention relates to compositions of matter and processes of preparing the same, and more particularly to the manufacture of products containing coal.

Various bituminous products are now in common use for coating purposes, particularly for the protection of metal against corrosion or of wood against decay and for coating concrete, brick, stone surfaces, etc. Many bituminous products have serious disadvantages. Usually it is necessary to heat or melt them prior to application and the fumes which result from this procedure are annoying to workmen and even dangerous, particularly if the work is done in closed rooms, as for instance in ships' holds.

Furthermore, in most cases it is necessary to prime the surface to be coated in order to make the bituminous material adhere thereto. It is also somewhat difficult to evenly apply the molten viscous products. The final coatings often show a tendency to run or to produce rough surfaces.

An object of the present invention is to provide an improved protective coating material and a method of preparing the same.

In accordance with the present invention, a coal product of a plastic nature is prepared from solutions of coal in tars and oils by the addition thereto of low boiling organic liquids which act as coagulating reagents. A product may be prepared which may be of a gel nature and which may assume a gelatinous or jelly state. A gel is a form of plastic and the term is herein intended to refer to a colloidally dispersed structure consisting of a solid and a liquid phase or also of two viscous liquid phases, and having shape and cohesion, and elastic properties, although it may be very rich in liquid.

The product of this invention differs from the product described in a copending application of H. J. Rose and W. H. Hill, Serial No. 393,124, filed Sept. 16, 1929, partly in that the latter product is a so-called non-evaporative coagulated coal solution, that is, one from which the coagulating agent evaporates very slowly or not at all, whereas the product of the present invention is one which

dries out and hardens by evaporation of the coagulating agent.

As set forth in the copending application Serial No. 97,467, filed March 25, 1926, by Rose and Hill, coal may be dissolved in oils such as coal tar or water-gas tar and certain distillates therefrom. The coal and oil are brought together and heated at normal or only moderately elevated pressures and moderately elevated temperatures of from about 200° C. to about 400° C. A given coal is heated with the solvent to non-decomposing temperatures, or in other words, below the temperature at which substantial chemical decomposition of the coal takes place.

Substantially all of the coal dissolves, forming homogeneous solutions which remain stable at temperatures below the point of rapid volatilization or even below the dissolving temperatures. The coals most easily dissolved in such solvents are generally the coking coals. Substantially all of such coals are soluble, the insoluble portions consisting of the mineral matter or ash and the mineral charcoal or fusain which may be present in limited amounts.

Preferably a high boiling coke-oven-tar oil is used as a solvent for coal. Other oils such as cracked petroleum oils, and especially the higher boiling distillates thereof, may also be used.

A coal solution may be prepared by heating one part of coal, such as Pittsburgh seam coal, and about three parts of crude coke-oven tar, for instance, in a closed vessel heated directly to a temperature of about 300° C. Water and undesirable light oils are allowed to escape before the vessel is closed. The resulting product is allowed to cool and is discharged into containers at a temperature lower than the lowest boiling temperature (about 200° C.) of compounds contained therein.

In addition to the solvents for coal mentioned above, sulphur treated oils and tars described in the co-pending application of Rose and Hill Serial No. 354,694, filed April 12, 1929, may also be used.

In accordance with the present process, a coal solution is prepared by dissolving coal

in any of the solvents mentioned above and the low boiling organic liquid is added to the solution formed. Practically every organic volatile solvent can be used, such as 5 benzene, toluene, solvent naphtha, gasoline and turpentine, or any combination of such solvents may be added to the coal solution to produce a plastic or coagulated mass.

These low boiling organic liquids tend to 10 thin the coal solution when added in too large amounts. The proper proportion is easily determined by the consistency obtained. In other words, a thickened mass which is of a semi-solid, plastic, or gelatinous nature, is 15 obtained, depending on the amount of volatile solvent added.

The consistency of the final product depends also somewhat on the time of digestion 20 of the coal solution in the volatile solvent, on the temperature of the coal solution or of the volatile solvent when about to be mixed, on the temperature to which the resulting mixture is heated, and on the speed with which the coagulating agent is added.

25 Upon the addition of any of the above volatile coagulating agents to a coal solution, there results a formation of minute particles of undissolved coal in the coal solvent. A given mass of treated coal solution may 30 contain some dissolved coal and particles of undissolved coal, or it may contain little or no dissolved coal, in which case substantially all of the previously dissolved coal is changed to a suspensoid.

35 By way of example, coal plastics may be produced by any one of the following methods:

40 *Example 1.*—One hundred pounds of coal solution having a melting point lower than the boiling point of a volatile solvent, such as benzene, are heated to thin or liquefy the same. Then about twenty pounds of the volatile solvent are introduced slowly with heating and vigorous stirring or kneading until 45 a homogeneous mass is obtained. It is advantageous to carry this out in a closed container fitted with a reflux condenser. After the resulting product is cooled, it is ready for use.

50 *Example 2.*—One hundred pounds of coal solution having a melting point somewhat above the boiling point of the volatile solvent used, for instance about 121° C., are charged into an autoclave having an internal 55 stirrer, together with about thirty pounds of the volatile solvent, such as benzene. The autoclave is closed and the temperature brought up to about 200° C. while stirring the contents of the autoclave. Upon cooling, 60 the product is ready for use.

55 *Example 3.*—One hundred pounds of coal solution having a melting point somewhat above the boiling point of the volatile solvent used, for instance about 121° C., are 65 charged into a stationary autoclave, fitted

with an internal stirrer, and heated until fluid, for example, to 200° C. Then about thirty pounds of volatile solvent are slowly introduced under pressure, while stirring. Upon cooling, the product is ready for use. 70

75 *Example 4.*—One hundred pounds of coal solution having a melting point of about 101° C. are crushed and mixed with ten pounds of volatile solvent, such as benzene. The mixture is allowed to soak for some time and is then charged into a kneading machine. As soon as a uniform mass has been formed, an additional ten pounds of benzene are added and the kneading continued until the mass becomes homogeneous. The total amount of 80 solvent may be added at one time, instead of in two or more batches. The product can be used as such or it may be passed through a homogenizer or colloid mill or extrusion apparatus. 85

90 In cases where it is desired to obtain a coating of a higher melting point than the coal solution employed, it is advantageous to add to the volatile solvent used in preparing the coagulated product such highly coagulating agents as linseed oil, paraffin, etc., mentioned in the copending application of Rose and Hill, Serial No. 393,124, filed Sept. 16, 1929. Any desired proportions of the latter agents may be used. It is preferred to add 95 from 1% to 5% thereof with respect to the weight of coal solution used. The same amount of volatile solvent may be used as that given in the above examples. Upon the application of this product to a surface, the 100 volatile solvent evaporates leaving a coating of relatively high melting point.

105 Products of the preceding type are prepared in cases where conditions are such that it is impractical to prepare plastic products 105 from high melting coal solutions.

110 Plastic or coagulated masses produced in accordance with the present invention may vary in consistency from a liquid to a solid, and those particularly of a soft, buttery or a doughy consistency may be readily applied with a trowel, a putty knife or similar instrument without the use of heat. They are usually applied like a plaster or paste in thick 115 layers and permitted to dry out in place, producing a coating which comprises the original coal solution. After drying out, the surface of such a coating may be smoothed or sealed with the aid of hot irons of various shapes.

120 Various inorganic or organic materials 120 may be added to the coagulated coal solutions to produce masses of varying consistencies and to produce coatings of varying degrees of hardness. The added materials may be of a purely inert type, for example, fillers such as bentonite clay and sand, or pigments such as aluminum bronze and venetian red, or fibrous materials such as mineral wool, asbestos and cellulose fibres; or they may exert 125 some chemical or physical action upon the 130

coal solution after the evaporation of the volatile solvent, as for instance, sulphur or its compounds; or they may exert a beneficial influence upon the surface to which the plastic mass is applied, for example, corrosion inhibitors such as nitrogen bases (pyridine), chromates, etc. Any one of or any combination of the above materials may be added to the coagulated coal solution in any desired proportion.

In addition to the uses mentioned above, coagulated coal solutions may be used as filling or sealing materials, or they may be used as cold patches in road construction, for roofs or other waterproofing purposes, for impregnating purposes, in molding compositions, in tree surgery, cements, binders, putties, printers' inks, etc.

It is obvious that the coal solution to be coagulated must be selected with a view to the conditions to which the final coating is to be subjected. For instance, the raw material required for the coating of surfaces which are submerged in cold water, as ships' plates, differs from a material which is to be used for coating tanks which are subjected to the temperature of boiling water or for the coating of surfaces subjected to direct sun light.

In general, the coal solution should be so selected that its melting point lies well above the highest temperature to be encountered. At the same time, the temperature-susceptibility factor should be as low as possible in order to avoid brittleness when the temperature drops unusually low. This requirement is well met by coal solutions due to the fact that they have a lower susceptibility factor than the ordinary bituminous coatings.

The products of this invention are very easily applied to surfaces to be coated and they do not require primers even when they are applied to very cold surfaces. Furthermore, they produce coatings having great adhesive strength.

I claim as my invention:

1. A process of preparing bituminous products, which process comprises heating coal and oil together to non-decomposing temperatures of the coal, namely about 200° C. to 50 400° C., to form a homogeneous fluid mass of coal and oil, maintaining the said mass in a fluid state, and mixing with the said mass a volatile solvent containing at least one of a group consisting of benzene, toluene, solvent naphtha, gasoline and turpentine, in sufficient amount only to thicken the said fluid mass.

2. A process of preparing bituminous products, which process comprises heating coal and oil together in the form of a homogeneous fluid mass at a temperature below the temperature at which chemical decomposition of the coal takes place and mixing with the said fluid mass a volatile solvent containing at least one of a group consisting of

benzene, toluene, solvent naphtha, gasoline and turpentine, in sufficient amount only to increase the consistency of the said fluid mass.

3. A bituminous product comprising coal and oil which have been heated together to 70 non-decomposing temperatures of about 200° C. to 400° C. to form a homogeneous fluid mass of coal and oil, and a volatile solvent selected from a group consisting of benzene, toluene, solvent naphtha, gasoline, and turpentine in sufficient amount to form a thickened soft mass.

4. A bituminous product consisting of a thickened soft mass comprising a previously dissolved coal uniformly distributed in a solvent for the coal, and benzene in an amount insufficient to cause settling of the coal.

5. A process of preparing bituminous products, which process comprises heating coal and oil together to non-decomposing 85 temperatures of the coal, namely about 200° C. to 400° C. to form a homogeneous fluid mass of coal and oil and thickening the said fluid mass by adding a volatile solvent which if added in a relatively small amount will increase the consistency of the said fluid mass but if added in large amounts will thin the said fluid mass.

In testimony whereof, I have hereunto subscribed my name this 9th day of September, 1929.

WILLIAM H. HILL.

100

105

110

115

120

125

130